

# United States Patent

Brenner et al.

[15] 3,663,158

[45] May 16, 1972

[54] **METHOD OF DEPOSITING AN OXYMETHYLENE POLYMER FROM FORMALDEHYDE IN THE VAPOR FORM ON CELLULOSIC TEXTILES AND THE RESULTING PRODUCT**

[72] Inventors: **Walter Brenner, Teaneck, N.J.; Jagadish Chanda Goswami, New York; Barry A. Rugg, Bronx, both of N.Y.**

[73] Assignee: **The United States of America as represented by the Secretary of Agriculture**

[22] Filed: **May 12, 1970**

[21] Appl. No.: **23,163**

[52] U.S. Cl. .... **8/116.4, 8/116.2, 8/120, 8/129, 8/DIG. 11, 8/116.3, 252/438, 8/149.2, 117/106**

[51] Int. Cl. .... **D06m 13/14, D06m 13/54, D06m 13/42**

[58] Field of Search .... **8/116.4, 116.2, 120, 116.3, 8/129**

[56]

**References Cited**

**UNITED STATES PATENTS**

3,545,913 12/1970 Joarder et al. .... **8/116.4**

**OTHER PUBLICATIONS**

Joarder et al., *Textile Research Journal*, 39, 49- 54 (1969).

*Primary Examiner*—George F. Lesmes

*Assistant Examiner*—J. Cannon

*Attorney*—R. Hoffman and W. Bier

[57]

**ABSTRACT**

Highly purified anhydrous monomeric formaldehyde vapor was prepared for immediate deposition on the surface of fibers of cotton. The process produced fabrics with enhanced physical properties with the deposition of oxymethylene polymer with molecular weights up to 18,000 and without significant crosslinking of the cellulosic chains. Supplementary treatments were applied to the oxymethylene polymer treated fabrics to further enhance the textiles with various desirable “-wash-wear” characteristics.

**4 Claims, 5 Drawing Figures**



FIG. 1

INVENTORS  
 WALTER BRENNER  
 JAGADISH CHANDRA GOSWAMI  
 BARRY A. RUGG

BY

*R. Hoffman*  
 ATTORNEY

PATENTED MAY 16 1972

3,663,158

SHEET 2 OF 5



FIG. 2

INVENTORS  
WALTER BRENNER  
JAGADISH CHANDRA GOSWAMI  
BARRY A.RUGG

BY

*R. Hoffman*

ATTORNEY



FIG. 3

INVENTORS  
WALTER BRENNER  
JAGADISH CHANDRA GOSWAMI  
BARRY A. RUGG

BY

*R. Hoffman*  
ATTORNEY



FIG. 4

INVENTORS  
WALTER BRENNER  
JAGADISH CHANDRA GOSWAMI  
BARRY A. RUGG

BY

*R. Hoffman*

ATTORNEY



FIG. 5

INVENTORS  
WALTER BRENNER  
JAGADISH CHANDRA GOSWAMI  
BARRY A. RUGG

BY

*R. Hoffman*

ATTORNEY

**METHOD OF DEPOSITING AN OXYMETHYLENE POLYMER FROM FORMALDEHYDE IN THE VAPOR FORM ON CELLULOSIC TEXTILES AND THE RESULTING PRODUCT**

A non-exclusive, irrevocable, royalty-free license in the invention herein described, throughout the world for all purposes of the United States Government, with the power to grant sublicenses for such purposes, is hereby granted to the Government of the United States of America.

This invention relates to a novel process for the formation and deposition of oxymethylene polymers from formaldehyde monomer in the vapor form on cellulosic textiles and to the composite polymeric products resulting from said process.

A very substantial effort has been made in the past and is continuing towards developing cellulosic textiles with a superior balance of performance properties, particularly so as regards the realization of durable wrinkle resistance or so-called "wash-wear" characteristics while retaining tensile and tear strength, abrasion resistance, the unique comfort factor and other desirable qualities of cellulosic textiles, in order to better meet specific consumer requirements. The treatment of cellulosic textile materials with formaldehyde or formaldehyde donors has long been experimented with for obtaining a more desirable balance of cellulosic textile properties. Given suitable reaction conditions, formaldehyde treatments result in crosslinking of cellulosic chains and the development of marked wrinkle resistant properties but other important physical characteristics including tensile strength, tear strength, elongation, and abrasion resistance are adversely affected. Typically, tensile strength losses amount to as much as 50-60 percent or greater. The loss in certain important physical properties associated with the strength and durability of the many formaldehyde-treated cellulosic textiles may be related to the nature of the generally strongly acidic catalysts and/or substantially elevated treatment temperatures—reaction conditions which attack the cellulose as well as to the short cross-links formed.

Accordingly, it is an object of the present invention to treat cellulosic materials with formaldehyde in such a manner that certain desirable physical properties such as tensile strength, elongation, tear strength, abrasion resistance, hand and appearance are significantly improved.

Another object is to treat cellulosic fabrics with formaldehyde so as to produce uniform and even oxymethylene polymer deposits onto the cellulose fiber surfaces without significantly altering such desirable physical properties as tensile strength, elongation, tear strength, abrasion resistance, hand and appearance.

A further object is to treat cellulosic fabrics with formaldehyde so as to produce uniform and essentially continuous oxymethylene polymer deposits on cellulose fibers without effecting any significant amount of crosslinking of the cellulosic chains.

An additional object is to treat the oxymethylene polymer-coated cellulosic textiles in such a manner that wash and wear characteristics can be achieved without the large decreases in important physical strength and durability characteristics generally associated with formaldehyde-treated cellulosic textiles.

Yet another object is to obtain modified oxymethylene polymer-coated cellulosic textiles with a superior balance of "wash-wear" characteristics and physical strength, durability properties and appearance than hitherto attainable.

A still further object is to obtain such modified oxymethylene polymer-coated cellulosic textiles with a superior balance of "wash-wear" characteristics and physical strength, durability properties and appearance using only low cost and therefore economically attractive treating agents and procedures.

Yet another further object is to obtain such modified oxymethylene polymer coated cellulosic textiles with a superior balance of "wash-wear" characteristics and physical strength, durability properties and appearance with treating agents and techniques amenable to continuous processing.

Still another additional object is to obtain such modified oxymethylene polymer coated cellulosic textiles with a superior balance of "wash-wear" characteristics and physical strength, durability properties and appearance which are permanently stabilized.

Still further objects and the entire scope of applicability of the present invention will become apparent from the following detailed descriptions; it should be understood, however, that the detailed descriptions and physical examples while indicating preferred embodiment of this invention are given by way of illustration only since many possible changes and modifications within the scope of this invention will become apparent to those skilled in the art from these detailed descriptions.

It has now been found that these objects can be obtained by utilizing the specific procedures to be discussed hereafter. Basically, these procedures include two reactions. The first one is the reaction of formaldehyde with cellulose under conditions which result in the formation of uniform and essentially continuous oxymethylene polymer deposits on cellulose fibers without significant crosslinking of the cellulose chains. This is accomplished by treating cellulosic fabrics with strictly anhydrous monomeric formaldehyde vapor under basic catalytic conditions. The oxymethylene polymer deposits formed may optionally be stabilized against thermal "unzipping" by end capping the oxymethylene hydroxyl end groups with acetic anhydride or other suitable reagents. The second step involves the treatment of the oxymethylene polymer-coated cellulosic fibers with one of the large and still growing number of cellulose crosslinking agents and particularly that group which have become known as the methylol amides. Quite conventional crosslinking textile finishing technology can be employed for this processing step. During the second step there is developed a substantial increase in both wet and dry wrinkle recovery with only relatively minimal effects on other important cellulose fabric properties including tensile and tear strengths, elongation, abrasion resistance and appearance. The resulting better overall balance of the treated cellulose fabric's performance properties is attributed to the presence of the uniform and essentially continuous tough oxymethylene polymer deposits on the cellulosic fibers obtained in the first processing step. By obvious appropriate modifications of this invention, cellulosic fabrics can be pleated or creased after the fabrics have been converted into apparel, etc.

The advantageous balance of properties imparted by the processes of the present invention including greatly improved wet and dry wrinkle recovery values and a high degree of retention of the desirable tensile strength, tear strength, elongation, abrasion resistance and appearance are all permanently embedded in the fabric. Thus, these properties have proven stable for in excess of 10 washings.

As previously described the present invention enables the deposition of uniform and essentially continuous coatings of oxymethylene polymer from gaseous monomeric formaldehyde and the subsequent crosslinking of the polymer-coated cellulose fibers with any of the many available cellulose crosslinking agents with particular emphasis but not in any way limiting on the industrially used methylol amides. The present invention effectively overcomes the most deleterious effects of the conventional cellulose crosslinking agents on cellulose textile by applying them to such oxymethylene polymer coated cellulose composite. While the mode of action of this invention is not entirely clear and we do not wish to be bound by any one explanation of the observed experimental fact, it is suggested that the presence of the physically tough and continuous oxymethylene polymer coatings on the cellulose fibers in some way mitigates the well known undesirable effects of these cellulose crosslinking agents.

As the cellulosic fabric there can be employed cotton, linen, hemp, ramie, sisal, rayons, and cellulose esters and/or ethers as well as mixtures of these fabrics with each other and/or synthetic fabrics including polyamides, polyesters, and acrylics. The invention is considered to be particularly applicable to the treatment of cotton fabric material such as cotton cloth.

In accordance with the above discussions, therefore, this invention comprises a formaldehyde monomer based vapor phase polymerization process more specifically comprising the exposure of suitably catalyzed cellulosic cloths to purified anhydrous formaldehyde vapor which then polymerizes to high molecular weight polyoxymethylene even at ambient temperatures selectively onto the catalyzed cellulosic surfaces to produce a uniform and essentially continuous oxymethylene polymeric coating thereon. Also, as noted earlier as a second processing step, it involves the treatment of such polyoxymethylene coated cellulosic surfaces with one of the many available cellulose crosslinking agents and with a controlled amount of crosslinking exhibiting a superior balance of performance properties including substantially higher dry and wet wrinkle recovery values without incurring the so undesirable marked losses in tensile strength, tear strength, elongation, abrasion resistance, etc. characteristic of conventionally treated crosslinked cellulosic fabrics.

Initially, high molecular weight polyoxymethylene polymer deposits are obtained by the immersion of cellulosic fabrics into a suitable alkaline catalyst solution at ambient temperatures and in air and then exposing the catalyzed cloths to purified anhydrous monomeric formaldehyde vapor. The time lag between the catalyst immersion process and the exposure of the catalyzed cellulosic cloth to the purified anhydrous monomeric formaldehyde vapor is not critical and conveniently may amount to between 5 and 15 minutes for many experiments. A typical catalyst system consists of a tertiary amine in the presence of a suitable amount of an anti-oxidant dissolved in a halogenated solvent. A preferred embodiment of such a catalyst system comprises a solution of tributylamine and diphenylamine antioxidant dissolved in carbon tetrachloride. The purified monomeric anhydrous formaldehyde vapor can be obtained in any number of well known ways, one preferred method being its generation from heating a paraformaldehyde-paraffin slurry at 115°-120° C. This formaldehyde gas generation is preferably conducted under inert conditions such as dry nitrogen gas. Purified anhydrous formaldehyde vapor is then carried in dry nitrogen gas to a polymerization chamber containing the catalyzed cellulosic cloths. Constructional features of the polymerization chamber and associated physical equipment set up will be described below and are shown in FIG. 1 of the accompanying drawing.

Oxymethylene polymer coatings are then deposited onto the surfaces of the cellulosic fibers in amounts depending upon such reaction variables as formaldehyde vapor concentration, reaction time, temperature, etc. Polymer deposits ranging from as little as 2 percent or less to in excess of 50 percent based on the weight of the cellulosic fabric are readily and reproducibly obtained by appropriate variations of the above referred to significant reaction variables. Typically, 10 percent polymer add-on's can be obtained in approximately 10 minutes exposure time to the formaldehyde vapor with one rather convenient set of reaction conditions. No cellulose crosslinking occurs as evidenced by solubility of the cellulosic substrate in solvents, such as cupriethylenediamine.

As is well known, the thermal stability of oxymethylene polymers is substantially enhanced by end capping their residual hydroxyl end groups to retard high temperature depolymerization or "unzipping," a reaction which can lead to the evolution of formaldehyde gas. One convenient and widely used procedure involves the esterification reaction of the oxymethylene polymer hydroxyl end groups with acetic anhydride. Other end-capping treatments include etherification with alcohols, reactions with chloroalkylethers and reactions with epoxides or isocyanates. If desired, this can be accomplished with the oxymethylene polymer-coated cellulosic fabrics by heating them in acetic anhydride solutions. A typical set of reaction conditions for such end-capping treatments involves heating the polymer-coated cellulosic fabrics in acetic anhydride solutions for approximately 30 minutes at 140° C. in the presence of a small amount of an esterification catalyst in order to speed up the esterification reaction. This

treatment reduces the solubility of the cellulosic substrates in solvents such as cupriethylenediamine.

The uncapped polyoxymethylene coatings can be removed from the cellulosic fibers by solvent extraction in hot 5 dimethylformamide followed by precipitation at ambient temperatures, purification by washing and, finally, vacuum drying. The chemical composition can be confirmed quite readily by means of infrared analysis. Melting point determinations and 10 other physical property measurements can also be carried out for identification purposes. Experiments can also be carried out involving the dissolution of the cellulose in cupriethylenediamine solvent leaving behind shells of polyoxymethylene polymer. These studies, which confirm the 15 absence of any chemical reaction between the oxymethylene polymer deposits and the cellulosic textiles and also demonstrate that no cellulose crosslinking has occurred, are further clarified by FIGS. 2 and 3 of the accompanying drawing. FIGS. 2 and 3, for example, compare the infrared spectra of a 20 commercial oxymethylene polymer film with an extracted oxymethylene polymer deposit from a coated cotton type cellulosic textile. The longitudinal photomicroscopic view of the oxymethylene polymer shows shells remaining after immersion of oxymethylene polymer-coated cotton cloths with various 25 amounts of polymer coating add-on's in cupriethylenediamine solvent. Similar studies have also been carried out with so-called end-capped oxymethylene polymer-coated cellulosic textiles. The results of the solvent extractions 30 are similar to the ones described immediately above, except that the cellulose substrate solubility in cupriethylenediamine is significantly reduced. Typical oxymethylene polymer extraction producers involve a 2-hour refluxing period in dimethylformamide. The end-capped polymer is extracted by refluxing for 6 hours in dimethylformamide.

Photomicrographic studies have also been made in order to 35 ascertain the location of these oxymethylene polymer deposits on the cellulosic textiles. Differential staining of the cross section of fiber specimens shows that the polymer deposits are located along the outer periphery of the fibers. A blue dispersion dye, Setacyl Blue 2 GS conc. 250 percent, was employed 40 to stain the oxymethylene polymer-coated cotton cloth samples and photomicrographic cross sections were studied.

The following examples illustrate processes for the deposition 45 of such oxymethylene polymer deposits from formaldehyde monomer in the vapor phase on cellulosic textiles.

#### EXAMPLE 1

Cotton print cloths 80 × 80 desized, bleached, and mercerized 50 were obtained and cut into 10-inch × 6-inch fabric samples for use in the vapor phase polymerization studies, which are described below. Suitably conditioned cloth samples were catalyzed by immersing in a catalyst solution comprising 7.5 cc. of tributylamine and 3.6 grams of diphenylamine dissolved in 1,500 cc. of carbon tetrachloride for 1 minute. The catalyzed conditioned cotton cloth samples were then exposed to purified anhydrous formaldehyde vapor in a 55 specially constructed vapor phase polymerization chamber for predetermined time periods. The formaldehyde vapor was generated by heating a slurry of paraformaldehyde in paraffin oil prepared by mixing thoroughly 75 grams of paraformaldehyde with 300 ml. of paraffin oil in a half liter resin kettle.

A general schematic diagram of the apparatus employed, 60 from which was derived the bulk of the experimental data of this invention and which demonstrates the manner in which the vapor phase coating of cotton cloth samples with polyoxymethylene is carried out most successfully, is depicted in FIG. 1 of the accompanying drawing.

70 Referring with more particularity to FIG. 1, the flow of gases is generally from left to right. The nitrogen cylinder 11 provides the inert propellant gas upon opening valve 12. The nitrogen gas passes through drying tube 13 and the rate of flow is measured by rotometer 14. The dried gas then passes via tube 15 through three-way valve 16 which was installed so as

to provide pressure readings through the use of mercury manometer 17, and then passes through sintered glass disc 19 into half-liter Pyrex resin kettle 21 which contains the paraformaldehyde and oil slurry 20. The kettle is covered tightly and heated by heating mantle 22. The thermometer 18 provides measurement of the temperature of the slurry.

The oxymethylene produced in the kettle is let out through water-jacketed condenser 23 when stopcock 24 is in the open position and thence passes through tube 26 into first trap 29 via inner tube 28 which connects to the trap through flexible tube 27. First trap 29 is immersed in a first Dewar flask 30 which contains coolant 31 consisting of ammonium chloride and ice.

Second trap 34 is immersed in a second Dewar flask 32, being cooled by a second coolant 33, identical to coolant 31, and receives the oxymethylene through tube 35 into the trap and out through tube 37 via flexible connector 36.

The three-way stopcock 38 controls the flow of argon, provided by argon cylinder 42, through tube 40 when valve 41 is opened. The manipulation of three-way stopcock 38 serves to provide the inert gas which evacuates the vapor phase polymerization chamber 45 as the gases would flow through straight external tube 43 which leads to the chamber through inner dispenser tube 44 when stopcock 38 is turned so as not to let gases out through outlet 39 which leads to an absorber hood (not shown).

The vapor phase polymerization chamber 45 is designed to hold cloth samples 47 suspended by sample holders 46, and the exhausted gases are let out to absorber hood (not shown) through outlet 48 after the reaction is complete.

The vapor phase polymerization chamber 45 employed in this experiment consisted of an 8-inch  $\times$  8-inch  $\times$  12-inch stainless steel-lined vacuum oven. The cloth samples 47 were mounted on stainless steel frames, which were then suspended inside the polymerization chamber from a sample holder 46, also constructed from stainless steel. A second chamber consisted of a half liter Pyrex resin kettle 21, which was jacketed with an electric heating mantle 22. This kettle contained the paraffin oil-paraformaldehyde slurry 20 from which the formaldehyde monomer vapor was generated by heating to 115°-120° C. The monomer was carried to the polymerization unit in dry nitrogen gas from nitrogen cylinder 11.

Water, methanol, and formic acid—the usual byproducts from the pyrolysis of paraformaldehyde—are known to cause considerable polymerization of monomeric formaldehyde leading to water soluble low molecular weight products. The nitrogen-formaldehyde gas stream was, therefore, purified by successive passage through two traps, namely, traps 29 and 34, cooled to -15° to -17° C. by respective coolants 31 and 33 consisting of ammonium chloride and ice, in order to condense such undesirable byproducts.

The polymerization chamber 45 containing the catalyzed cotton cloth samples 47 was flushed with argon gas from argon cylinder 42 in order to displace air before admitting the purified formaldehyde-nitrogen gas stream. This gas mixture was then directed into the chamber, thus causing polymerization of the formaldehyde vapor onto the surfaces of the catalyst activated cotton cloth samples. Excess reagent gas mixture left the polymerization chamber 45 through outlet 48 and was condensed in a cold trap.

Typical specific reaction conditions included a nitrogen gas flow rate, as measured by rotometer 14, in the order of 0.8 to 1.2 liters/min., a paraformaldehyde-paraffin oil slurry temperature of 115°-120° C. as measured by thermometer 18 and a polymerization chamber temperature of 25° C. The exposure time of the catalyst activated cloth samples to the purified monomer formaldehyde vapor was varied in order to obtain different polymer add-on's and to ascertain such effects on the pertinent physical and chemical properties of the cotton samples. Experimental results relating the exposure time of the catalyst cotton cloth samples to the oxymethylene polymer add-on's are shown in FIG. 4 of the accompanying drawing.

The oxymethylene polymer coating was recovered from the cotton cellulose substrate by extraction in refluxing dimethylformamide for 2 hours followed by precipitation at ambient temperatures, filtering, washing with acetone and ether and vacuum drying at 50° C. Thin films of polymer were prepared by pressing an appropriate amount of the dried recovered polymer at 30° C. in a laboratory press. Identification was accomplished by comparing an infrared spectrograph of this material with that of a commercially produced polyoxymethylene film. Melting point was 165° C. The data obtained were analogous to the information presented in FIGS. 2 and 3 of the accompanying drawing, except for the absence of C = O groups introduced in the commercial product by end capping via esterification with acetic anhydride. The relative viscosity of the recovered polyoxymethylene was determined in a viscometer utilizing a 0.5 percent solution of oxymethylene polymer at 60° C. in p-chlorophenol containing 2 percent by weight of alpha pinene. The inherent viscosity was calculated from the equation: inherent viscosity =  $\ln \frac{relative\ viscosity}{C}$  where relative viscosity = solution viscosity/solvent viscosity, C = concentration of solute in solution (grams polymer per 100 ml. of solution). It was found to be 0.865. The inherent viscosity was then related to the molecular weight using the expression inherent viscosity =  $3.82 \times 10^{-4} M_n^{0.83}$ . The molecular weight ( $M_n$ ) calculated in this manner was approximately 11,000-12,000.

Pertinent physical properties of oxymethylene polymer-coated 80  $\times$  80 cotton print cloth are summarized in Table 1 as a function of polymer add-on. The data show not only retention but even some improvement in abrasion resistance and tear strength, etc. As expected, wrinkle recovery values were not changed by this polymer deposition process in which neither the vapor phase deposited polyoxymethylene nor the cellulose substrate were crosslinked. This example demonstrates the retention and even shows some improvement in selected important physical properties of the oxymethylene coated cotton cloths prepared in accordance with the teachings of this invention.

#### EXAMPLE 2

Cotton print cloths 80  $\times$  80 desized, bleached and mercerized were obtained and cut into 10-inch  $\times$  6-inch fabric samples for use in formaldehyde vapor phase polymerization studies. The cloth samples were conditioned and catalytically activated in the same manner as described in Example 1. The catalyzed cotton cloth samples were then exposed to formaldehyde vapor again generated by heating a slurry of paraformaldehyde in paraffin oil to 115°-120° C. The experimental setup was identical with the one shown schematically in FIG. 1 and discussed in Example 1 above, except that the formaldehyde vapor bypassed the two low temperature traps 29 and 34 and was fed directly into the polymerization chamber 45.

Polymer deposition occurred on the catalyzed cloth samples 47 in the same manner as before. The polymer deposits were, however, found to be readily water soluble and could thus be easily removed from the cloth samples. Further studies showed that the polymer deposits, which were found to be of quite low molecular weight (below 1,000), did not significantly affect any of the pertinent physical or otherwise important properties of the cotton cloth samples. This experiment shows the importance of purifying the formaldehyde monomer by removal of the byproducts of the paraformaldehyde pyrolysis including water, methanol, and formic acid, in order to produce high molecular weight oxymethylene polymer.

#### EXAMPLE 3

Cotton print cloths, 80 $\times$ 80 desized, bleached, and mercerized were obtained and again cut into 10-inch  $\times$  6-inch fabric samples for use in additional vapor phase polymerization studies. These were conducted with the same equipment and employing analogous chemical reagent and procedures as

described in Example 1 except that the time of immersion of the cotton print cloth in the catalyst solution was varied. The results in terms of polymer add-on per time unit are shown in Table 2. Immersion time of the cotton print cloth into the carbon tetrachloride catalyst solution is apparently not a primary variable for the polymer deposition process described in Example 1.

#### EXAMPLE 4

Cotton print cloths, 80 × 80 desized, bleached, and mercerized were obtained and cut into 10-inch × 6-inch fabric samples for use in vapor phase polymerization studies. In order to study the effects of polymerization temperature on polymer deposition a series of experiments were run during which the temperature in the vapor phase polymerization chamber 45 was varied between 15° and 60° C. All other procedures and materials were the same as described in Example 1 above.

It was found that polymerization temperatures in the order of 15° C. resulting in substantially lower polyoxymethylene deposition rates amounted to approximately one-half of the data presented in Example 1. However, the molecular weight of the polymer deposits was significantly higher. Using previously outlined procedures, it was determined to be in the order of 17,000-18,000. Pertinent properties of the oxymethylene polymer-coated cotton cloths were quite similar to the ones obtained when polymerization was effected at approximately 25° C. Experiments carried out at 60° C. failed to yield any substantial polymer deposit thus suggesting the existence of a ceiling temperature for the vapor phase formaldehyde polymerization given in the above-detailed experimental conditions.

As indicated, the second step of the above-outlined processing sequence involves the treatment of the oxymethylene polymer cellulosic fabrics with one of the many available large and still growing number of cellulose crosslinking agents and particularly a compound selected from that group of chemicals, which have become known as the methylol amides. While oxymethylene polymer-coated cellulosic fabrics obtained from the vapor phase polymerization of anhydrous formaldehyde onto a cellulosic substrate have been experimentally shown to exhibit certain desirable improved physical strength properties, including tensile strength elongation, tear strength, abrasion resistance, they require substantially enhanced shape holding properties such as wrinkle resistance, wash-wear characteristics and dimensional stability, to enhance their utility in volume apparel applications. It is the purpose of this secondary treatment to develop such properties with polyoxymethylene coated fabrics.

TABLE 2

Effect of Catalyst Immersion Time on Polymer Add-On  
(formaldehyde vapor phase polymerization at 25° C.)

|    | Sample                                                                                                                                                                                                                                                                                                                                                                                                                                                                                                                                                                                                                                                                             | Immersion Time (sec.) | Exposure Time (min.) | % Polymer Add-On |
|----|------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-----------------------|----------------------|------------------|
| 10 | A-1                                                                                                                                                                                                                                                                                                                                                                                                                                                                                                                                                                                                                                                                                | 30                    | 10                   | 4.5              |
|    | B-1                                                                                                                                                                                                                                                                                                                                                                                                                                                                                                                                                                                                                                                                                | 60                    | 10                   | 5.5              |
|    | C-1                                                                                                                                                                                                                                                                                                                                                                                                                                                                                                                                                                                                                                                                                | 120                   | 10                   | 6.0              |
|    | D-1                                                                                                                                                                                                                                                                                                                                                                                                                                                                                                                                                                                                                                                                                | 300                   | 10                   | 3.3              |
|    | E-1                                                                                                                                                                                                                                                                                                                                                                                                                                                                                                                                                                                                                                                                                | 600                   | 10                   | 5.7              |
|    | F-1                                                                                                                                                                                                                                                                                                                                                                                                                                                                                                                                                                                                                                                                                | 1200                  | 10                   | 4.2              |
| 15 | A-2                                                                                                                                                                                                                                                                                                                                                                                                                                                                                                                                                                                                                                                                                | 30                    | 20                   | 15.0             |
|    | B-2                                                                                                                                                                                                                                                                                                                                                                                                                                                                                                                                                                                                                                                                                | 60                    | 20                   | 13.5             |
|    | C-2                                                                                                                                                                                                                                                                                                                                                                                                                                                                                                                                                                                                                                                                                | 120                   | 20                   | 16.0             |
|    | D-2                                                                                                                                                                                                                                                                                                                                                                                                                                                                                                                                                                                                                                                                                | 300                   | 20                   | 15.0             |
|    | E-2                                                                                                                                                                                                                                                                                                                                                                                                                                                                                                                                                                                                                                                                                | 600                   | 20                   | 14.2             |
|    | F-2                                                                                                                                                                                                                                                                                                                                                                                                                                                                                                                                                                                                                                                                                | 1200                  | 20                   | 13.9             |
| 20 | A-2                                                                                                                                                                                                                                                                                                                                                                                                                                                                                                                                                                                                                                                                                | 30                    | 30                   | 20.0             |
|    | B-3                                                                                                                                                                                                                                                                                                                                                                                                                                                                                                                                                                                                                                                                                | 60                    | 30                   | 21.5             |
|    | C-3                                                                                                                                                                                                                                                                                                                                                                                                                                                                                                                                                                                                                                                                                | 120                   | 30                   | 23.0             |
|    | D-3                                                                                                                                                                                                                                                                                                                                                                                                                                                                                                                                                                                                                                                                                | 300                   | 30                   | 19.0             |
|    | E-3                                                                                                                                                                                                                                                                                                                                                                                                                                                                                                                                                                                                                                                                                | 600                   | 30                   | 20.7             |
|    | F-3                                                                                                                                                                                                                                                                                                                                                                                                                                                                                                                                                                                                                                                                                | 1200                  | 30                   | 22.5             |
| 25 | A-2                                                                                                                                                                                                                                                                                                                                                                                                                                                                                                                                                                                                                                                                                | 30                    | 30                   | 20.0             |
|    | B-3                                                                                                                                                                                                                                                                                                                                                                                                                                                                                                                                                                                                                                                                                | 60                    | 30                   | 21.5             |
|    | C-3                                                                                                                                                                                                                                                                                                                                                                                                                                                                                                                                                                                                                                                                                | 120                   | 30                   | 23.0             |
|    | D-3                                                                                                                                                                                                                                                                                                                                                                                                                                                                                                                                                                                                                                                                                | 300                   | 30                   | 19.0             |
|    | E-3                                                                                                                                                                                                                                                                                                                                                                                                                                                                                                                                                                                                                                                                                | 600                   | 30                   | 20.7             |
|    | F-3                                                                                                                                                                                                                                                                                                                                                                                                                                                                                                                                                                                                                                                                                | 1200                  | 30                   | 22.5             |
| 30 | A cellulose crosslinking binding treatment is considered generally necessary to advance shape-holding properties of cellulosic textiles employing conventional textile finishing technology. The base catalyzed polyformaldehyde vapor phase polymerization process as developed does not involve chemical reaction with the cellulosic substrate and given the thermoplastic character of the polymer, would not be expected to show any significant improvements in wrinkle recovery, dimensional stability and other indications of improved fabric shape-holding ability. The application of a crosslinking finishing treatment would therefore seem to be very much in order. |                       |                      |                  |
|    | 35                                                                                                                                                                                                                                                                                                                                                                                                                                                                                                                                                                                                                                                                                 |                       |                      |                  |
|    | 30                                                                                                                                                                                                                                                                                                                                                                                                                                                                                                                                                                                                                                                                                 |                       |                      |                  |
|    | 35                                                                                                                                                                                                                                                                                                                                                                                                                                                                                                                                                                                                                                                                                 |                       |                      |                  |
|    | 30                                                                                                                                                                                                                                                                                                                                                                                                                                                                                                                                                                                                                                                                                 |                       |                      |                  |
|    | 35                                                                                                                                                                                                                                                                                                                                                                                                                                                                                                                                                                                                                                                                                 |                       |                      |                  |
| 40 | 40                                                                                                                                                                                                                                                                                                                                                                                                                                                                                                                                                                                                                                                                                 |                       |                      |                  |
|    | 45                                                                                                                                                                                                                                                                                                                                                                                                                                                                                                                                                                                                                                                                                 |                       |                      |                  |
|    | 45                                                                                                                                                                                                                                                                                                                                                                                                                                                                                                                                                                                                                                                                                 |                       |                      |                  |
|    | 50                                                                                                                                                                                                                                                                                                                                                                                                                                                                                                                                                                                                                                                                                 |                       |                      |                  |
|    | 50                                                                                                                                                                                                                                                                                                                                                                                                                                                                                                                                                                                                                                                                                 |                       |                      |                  |
|    | 50                                                                                                                                                                                                                                                                                                                                                                                                                                                                                                                                                                                                                                                                                 |                       |                      |                  |

TABLE 1

[Physical properties of polyoxymethylene coated cotton cloth samples]

| Sample designation | Percent weight gain <sup>a</sup> | Breaking strength, lb. <sup>b</sup> |                   |                    |                   | Abrasion (flex) resistance cycles-failure <sup>d</sup> |      |      |
|--------------------|----------------------------------|-------------------------------------|-------------------|--------------------|-------------------|--------------------------------------------------------|------|------|
|                    |                                  | Warp                                |                   | Fill               |                   | Tearing strength, g. <sup>c</sup>                      | Warp | Fill |
|                    |                                  | Percent elongation                  | Breaking strength | Percent elongation | Breaking strength |                                                        |      |      |
| Control.....       | 5.8                              | 58.7                                | 17.4              | 37.9               | 470               | 784                                                    | 87   |      |
| #1-C.....          | 8.5                              | 63.4                                | 20.1              | 34.0               | 578               | 870                                                    | 74   |      |
| #2-C.....          | 2.0                              | 8.0                                 | 60.6              | 20.8               | 588               | 908                                                    | 90   |      |
| #3-C.....          | 5.5                              | 7.4                                 | 60.1              | 20.9               | 59.9              | 902                                                    | 119  |      |
| #4-C.....          | 9.3                              | 7.4                                 | 56.6              | 20.3               | 30.0              | 552                                                    | 904  | 126  |
| #5-C.....          | 14.7                             | 7.1                                 | 61.5              | 19.1               | 38.0              | 540                                                    | 892  | 153  |
| #6-C.....          | 24.0                             | 6.3                                 | 66.2              | 16.3               | 41.1              | 432                                                    | 850  | 194  |

<sup>a</sup> Avg. value of 8 samples.

<sup>b</sup> Avg. value of 5 runs.

<sup>c</sup> Avg. value of 4 runs.

<sup>d</sup> Avg. value of 3 runs.

NOTE: Sample #1-C: Control treated with acetic anhydride at 140° C. for 30 min. Sample did not gain any weight. The coated samples were treated with acetic anhydride at 140° C. for 30 min.

Recognizing this situation, a series of experiments have been carried out in which oxymethylene polymer coated cellulosic fabrics were treated with various types of cellulose cross-linking agents and the resultant composite characteristics determined in terms of pertinent textile properties with emphasis on the development of shape-holding characteristics to be ascertained by tests such as dry and wet wrinkle recovery values. Considerable attention was paid to reproducibility of results necessitating the testing of many duplicate samples. Specific chemical types of crosslinking agents which were reacted with polyoxymethylene treated cellulosic fabrics included the following:

- a. methylol derivatives of cyclic ureas, methylol derivatives of melamine, methylol derivatives of urea, and methylol carbamates; an unbuffered glyoxal based reactant, and a reactant described as a nonresinous cyclic uron derivative;
- b. multifunctional carboxylic acids, e.g., maleic acid, 1,2,3,4 cyclopentanetracarboxylic acid; trimellitic acid; mellitic acid and 1,2,3,4 butanetracarboxylic acid;
- c. epichlorohydrin and difunctional epoxides.

Experimentally the indicated crosslinking finishing treatments were carried out by padding oxymethylene polymer coated cellulosic fabrics with suitable catalyzed aqueous solutions of these crosslinking agents followed by drying, heating, washing and drying in accordance with the specific procedures recommended by the manufacturer of the crosslinking agent employed. Typical crosslinking conditions for a methylolamide type crosslinking agent, for example, were the treatment of a cellulosic cloth coated with known amounts of polyoxymethylene, with aqueous solution comprising 5 weight percent of the active crosslinking agent, 1 percent catalyst, e.g.,  $Zn(NO_3)_2 \cdot 6H_2O$  or equivalent, 2 percent softener Mykon SF polyethylene emulsion or equivalent and 0.1 percent Triton X 405 alkylphenoxy ethanol or equivalent for approximately 10 minutes at ambient temperatures. The samples were then dried for 15 minutes in an air circulating oven at 80° C. Crosslinking was accomplished by heating the treated samples for predetermined time periods at temperatures selected in the 140°-165° C. range in a forced air draft oven. The samples were then washed, dried to constant weight, etc., and subjected to the various evaluation tests traditionally employed for crosslinking finishes.

Typical experimental data on the properties of some cross-linked polyoxymethylene coated cotton fabrics are described in the subsequent examples with the aid of both tables and graphs. It need scarcely be emphasized that considering the very large number of possible reaction variables which would all have to be explored to obtain a complete analysis of their interactions and effects with respect to the product properties these data illustrate trends only. It is understood that many possible changes and modifications are possible and will become apparent to those skilled in the art from these detailed descriptions of examples without departing from the scope of this invention.

Certain of the crosslinked oxymethylene polymer-coated cellulosic fabrics exhibit a substantially superior balance of performance properties compared to conventionally cross-linked cellulosic fabrics, particularly as regards strength retention, wrinkle recovery (wet and dry) and abrasion resistance qualities. This applies especially to selected methylol amide-type crosslinking agents including dimethylolethyleneurea which is marketed commercially under the trade name Rhonite R-1. Rhonite R-1 crosslinked oxymethylene-coated 80 × 80 print cloth cotton fabrics show strength retention as high as 80 percent over a wide range of crosslinking agent add-on's together with good wrinkle recovery values and satisfactory abrasion resistance. For comparison purposes conventionally Rhonite R-1 crosslinked cellulosic fabrics are characterized by a substantial gain in wrinkle recovery values—at the expense of strength losses of 50 percent or more as well as much lower abrasion resistance. These properties can be viewed as decreased apparel wearing qualities. Other widely used methylolamide crosslinking agents show a

similarly unsatisfactory behavior with cellulosic fabrics and definite improvements when they are applied to oxymethylene polymer-coated fabrics.

The reasons for the improved balance of properties resulting from the crosslinking of oxymethylene polymer-coated cellulosic fabrics are as yet not clearly understood. They are believed to be related to the physical and chemical properties of the tough polyoxymethylene deposits which surround the cellulose fibers. For conventionally crosslinked cellulose fabrics, strength losses increase sharply at larger add-on's of crosslinking agent. Above 12-15 percent add-on's strength retentions are frequently as low as 40 percent. The treatment sequence embodied in this invention is less sensitive to both polymer and crosslinking agent add-on's. For Rhonite R-1 crosslinked oxymethylene-coated fabrics, strength retentions remain in the order of 80 percent for a wide range of polymer add-on's to which varying amounts of crosslinking agents have been applied.

It is noteworthy that, as expected, all the crosslinked polyoxymethylene-coated cotton fabrics proved to be insoluble upon immersion in cuene. Experiments were also carried out to ascertain the thermal stability of these crosslinked polyoxymethylene-encapsulated cotton cloths. Elevated temperature tests conducted in accordance with previously described procedures demonstrated a degree of thermal stability which is indicative of crosslinking with end capping.

#### EXAMPLE 5

Oxymethylene polymer-coated 80 × 80 desized, bleached and mercerized cotton print cloths prepared as described in Example 1 and cut into 10-inch × 6-inch fabric samples, were conditioned and then padded with an aqueous solution comprising 5 weight percent Rhonite R-1 dimethylolethyleneurea, 1 weight percent of catalyst  $Zn(NO_3)_2 \cdot 6H_2O$ , 2 weight percent Mykon SF polyethylene emulsion softener and 0.1 weight percent Triton X-405 wetting agent for approximately 10 minutes at ambient temperatures. The padded textiles were then dried for 15 minutes at 80° C. in an air circulating oven. Curing or crosslinking was then carried out at the much higher temperature of 160°-165° C. for approximately 2-5 minutes. The crosslinked polymer-coated cotton samples were then washed, dried to constant weight and subjected to the conventional evaluation tests for crosslinked cellulosic fabrics. Typical results are summarized in Table 3 and are shown graphically in FIG. 5 of the accompanying drawing. The data are presented for crosslinking agent add-on's in the order of 2-4 percent; this information is given for oxymethylene polymer-coated fabrics containing up to 40 percent polymer.

The crosslinked oxymethylene polymer-coated cotton fabrics exhibit strength retentions as high as 80 percent up to approximately 40 percent polymer add-on's with only 2-4 weight percent Rhonite R-1 crosslinking agent. Good wrinkle recovery characteristics were obtained at relatively low add-on's together with satisfactory abrasion resistance. In contrast, the strength properties of conventional crosslinked uncoated cotton fabrics decrease sharply with greater polymer add-on's as shown clearly in FIG. 5.

#### EXAMPLE 6

Oxymethylene polymer-coated 80 × 80 desized, bleached and mercerized cotton print cloths prepared as described in Example 1 and cut into 10-inch × 6-inch fabric samples, were conditioned and then padded with an aqueous solution comprising 5 weight percent Aerotex Reactant LC unbuffered glyoxal-based reactant, 1 weight percent of catalyst  $Zn(NO_3)_2 \cdot 6H_2O$ , 2 weight percent Mykon SF polyethylene emulsion softener and 0.1 weight percent Triton X-405 wetting agent for approximately 10 minutes at ambient temperatures. The padded textiles were then dried for 15 minutes at 80° C. in an air circulating oven. Curing or crosslinking was then carried out at the much higher temperature of 160°-165° C. for approximately 2-5 minutes. The crosslinked polymer-coated cotton samples were then washed, dried to constant weight

and subjected to the conventional evaluation tests for cross-linked cellulosic fabrics. Typical results are summarized in Table 4 and are shown graphically in FIG. 6 of the accompanying drawing. The data are presented for crosslinking agent add-on's in the order of 2-4 percent; thus information is given for oxymethylene polymer-coated fabrics containing up to 40 percent polymer.

The crosslinked oxymethylene-coated cotton fabrics exhibit strength retentions in the order of 70 percent up to approx. 40 percent polymer add-on's with only 2-4 percent weight Aerotex Reactant LC crosslinking agent. Good wrinkle recovery characteristics were obtained at relatively low add-on's together with satisfactory abrasion resistance. In contrast the strength properties of conventionally crosslinked uncoated cotton fabric samples decrease sharply with greater crosslinking agent add-on's as is clearly also shown in FIG. 6.

#### EXAMPLE 7

This example explores the use of polyfunctional carboxylic acids for end capping the oxymethylene polymer coating and reaction with the cotton cellulose. Oxymethylene polymer-coated 80 × 80 desized, bleached and mercerized cotton print cloths prepared as described in Example 1 and cut into 10-inch × 6-inch fabric samples, were conditioned and then padded successively with two aqueous solutions. The first solution was comprised of 15 weight percent sodium acetate and 0.1 weight percent Triton X-100 wetting agent while the second one contained 2 weight percent of maleic acid. The cotton test samples were then dipped in the first solution for approximately 10 minutes in order to promote swelling of the cotton and facilitate the penetration of the esterification catalyst. After removal of excess solution, the samples were immersed in the solution of the maleic acid up to 10 minutes, dried at 80° C. for approximately 10 minutes and cured at selected temperatures ranging from 140°-160° C. for 15-20 minutes in an air-circulating oven. The samples were then washed, dried to constant weight, etc., and subjected to the customary fabric evaluation tests. Typical results are summarized in Table 5. These data show that unsatisfactory results were obtained with this treatment.

#### EXAMPLE 8

This example describes the application of another polycarboxylic acid for treatment with the oxymethylene polymer-coated cotton fabrics. Oxymethylene polymer-coated 80 × 80 desized, bleached and mercerized cotton print cloths prepared as described in Example 1 and cut into 10-inch × 6-inch fabric samples, were conditioned then padded successively with two aqueous solutions. The first solution was comprised of 15 weight percent sodium acetate and 0.1 weight percent Triton X-100 wetting agent, the second contained 2 weight percent of 1,2,3,4 cyclopentane tetracarboxylic acid. The cotton test samples were dipped in the first solution for approximately 10 minutes in order to promote swelling of the cotton and facilitate the penetration of the catalyst. After removal of excess solution, the samples were immersed in the solution of the acid for 10 minutes, dried at 80° C., then cured for 20 minutes at 150° C. in an air-circulating oven. The samples were then washed, dried to constant weight, etc., and subjected to the customary fabric evaluation tests.

Typical results are summarized in Table 6. These data illustrate clearly unsatisfactory results obtained with this treatment.

#### EXAMPLE 9

This example describes the treatment of oxymethylene polymer-coated cotton fabrics with epichlorohydrin. Oxymethylene polymer-coated 80 × 80 desized, bleached and mercerized cotton print cloths prepared as described in Example 1 and cut into 10-inch × 6-inch fabric samples were conditioned then were reacted with epichlorohydrin in the presence of an alkaline catalyst using a two dip procedure. Reaction conditions were arranged in such a manner that the polyoxymethylene polymer add-on's amounted to between 8 and 12

percent, based upon the initial weight of the conditioned cotton cloths. In the first process step, the samples were immersed in a 5 weight percent sodium hydroxide solution in absolute ethanol. Curing was accomplished in an air circulating oven at 100° C. for 10 minutes. The products were found to be insoluble in cuene.

Data are summarized in Table 7. It will be noted that only very low weight gains were obtained even though initial polyformaldehyde loadings of the cotton were quite substantial in certain cases. This indicates that the epichlorohydrin reaction degraded the polyoxymethylene under the specific experimental conditions employed. This treatment is therefore not suitable for the proposed aims of this invention. Based on the wrinkle recovery and strength retentions measured, the amount of crosslinking which had occurred, must have been limited. It is specialized that the main reaction occurred between the polyformaldehyde and the epichlorohydrin.

TABLE 3

Some physical properties of polyoxymethylene-coated cotton cloths treated with Rhonite R-1 crosslinking agent.

| Sample               | % Add-on <sup>(a)</sup> | Breaking Strength <sup>(b)</sup> (lb.) | % Elongation <sup>(b)</sup> | DWR <sup>(c)</sup> (W+F) | WWR <sup>(d)</sup> (W+F) |
|----------------------|-------------------------|----------------------------------------|-----------------------------|--------------------------|--------------------------|
| Control              | —                       | 43.5                                   | 21.5                        | 195                      | 185                      |
| C-A <sup>(e)</sup> 1 | 1.5                     | 24.0                                   | 22.0                        | 272                      | —                        |
| C-A 2                | 3.2                     | 19.8                                   | 21.9                        | 296                      | 279                      |
| C-A 3                | 3.6                     | 18.7                                   | 19.9                        | 317                      | —                        |
| C-A 4                | 1.5                     | 29.0                                   | 24.1                        | 284                      | 268                      |
| C-A 5                | 2.1                     | 23.0                                   | 19.3                        | 302                      | —                        |
| 231                  | 3.7                     | 38.3                                   | 23.2                        | 288                      | 270                      |
| 232                  | 6.8                     | 39.3                                   | 23.5                        | 271                      | 259                      |
| 265                  | 3.0                     | 26.7                                   | 23.2                        | 302                      | 285                      |
| 270                  | 13.3                    | 35.5                                   | 23.9                        | 248                      | 237                      |
| 271                  | 10.0                    | 28.8                                   | 22.3                        | —                        | —                        |
| 272                  | 9.6                     | 28.8                                   | 20.0                        | —                        | —                        |
| 225                  | 16.0                    | 35.8                                   | 19.0                        | —                        | —                        |
| 235                  | 18.7                    | 37.2                                   | 17.7                        | 196                      | 180                      |
| 236                  | 18.3                    | 33.8                                   | 18.2                        | 200                      | 175                      |
| 237                  | 22.1                    | 38.5                                   | 19.3                        | —                        | —                        |
| 238                  | 25.4                    | 48.0                                   | 22.9                        | 153                      | 140                      |
| 227                  | 27.0                    | 48.0                                   | 23.0                        | —                        | —                        |
| 310                  | 26.2                    | 32.8                                   | 16.4                        | —                        | —                        |
| 297                  | 33.6                    | 36.2                                   | 17.2                        | 151                      | 138                      |
| 320                  | 36.8                    | 38.8                                   | 15.8                        | —                        | —                        |

<sup>(a)</sup>Percent add-on represents the total weight gain due to the polyoxymethylene and the crosslinking agent after cure except those samples designated C-A, etc. (See footnote e).

<sup>(b)</sup>ASTM D1682-64; Average of three runs per sample, fill direction only.

<sup>(c)</sup>ASTM D1295-60-T; Average of three runs per sample.

<sup>(d)</sup>ASTM D1295-60-T; Average of three runs per sample; samples conditioned for five minutes in 0.1% Triton X-100 solution.

<sup>(e)</sup>Control samples treated with crosslinking agent only.

TABLE 4

Some physical properties of polyoxymethylene-coated cotton cloths treated with Aerotex React LC crosslinking agent.

| Sample               | % Add-on <sup>(a)</sup> | Breaking Strength <sup>(b)</sup> (lbs.) | % Elongation | DWR <sup>(c)</sup> (W+F) | WWR <sup>(d)</sup> (W+F) |
|----------------------|-------------------------|-----------------------------------------|--------------|--------------------------|--------------------------|
| Control              | —                       | 43.5                                    | 21.5         | 195                      | 185                      |
| C-B <sup>(e)</sup> 1 | 2.9                     | 27.2                                    | 23.2         | 298                      | —                        |
| C-B 2                | 1.7                     | 30.7                                    | 24.9         | 249                      | 234                      |
| C-B 3                | 1.5                     | 30.5                                    | 27.0         | 246                      | —                        |
| C-B 4                | 1.8                     | 27.2                                    | 22.7         | 254                      | 242                      |
| C-B 5                | 2.3                     | 24.2                                    | 21.4         | 300                      | 290                      |
| 326                  | 3.3                     | 41.2                                    | 25.6         | 232                      | 245                      |
| 327                  | 2.7                     | 40.2                                    | 27.5         | 217                      | 230                      |
| 328                  | 3.7                     | 43.7                                    | 27.1         | 205                      | 195                      |
| 313                  | 6.5                     | 31.5                                    | 20.0         | —                        | —                        |
| 325                  | 6.8                     | 32.3                                    | 22.4         | —                        | —                        |
| 244                  | 8.7                     | 30.0                                    | 19.1         | —                        | —                        |
| 303                  | 9.5                     | 44.3                                    | 27.7         | 187                      | —                        |
| 329                  | 12.5                    | 32.5                                    | 19.8         | —                        | —                        |
| 323                  | 15.9                    | 27.3                                    | 18.3         | 195                      | 178                      |
| 240                  | 17.3                    | 30.8                                    | 16.5         | —                        | —                        |

|     |      |      |      |     |     |     |     |    |     |   |
|-----|------|------|------|-----|-----|-----|-----|----|-----|---|
| 322 | 18.1 | 25.3 | 16.2 | —   | —   | 124 | 6.0 | 38 | 5.7 | — |
| 302 | 22.3 | 36.2 | 19.9 | 240 | 210 | 125 | 4.1 | 43 | 5.8 | — |
| 299 | 23.1 | 31.0 | 18.3 | —   | —   | 149 | 3.9 | 41 | 5.6 | — |
| 324 | 25.4 | 30.7 | 18.0 | —   | —   |     |     |    |     |   |
| 300 | 33.4 | 35.7 | 14.9 | 175 | 162 |     |     |    |     |   |

<sup>(a)</sup> Percent add-on represents the total weight gain due to the polyoxymethylene and the crosslinking agent after cure except those samples designated C-A, etc. (See footnote e).

<sup>(b)</sup> ASTM D1682-64; Average of three runs per sample, fill direction only.

<sup>(c)</sup> ASTM D1295-60-T; Average of three runs per sample.

<sup>(d)</sup> ASTM D1295-60-T; Average of three runs per sample; samples conditioned for five minutes in 0.1% Triton X-100 solution.

<sup>(e)</sup> Control samples treated with crosslinking agent only.

TABLE 5

### Some physical properties of polyoxymethylene-coated cotton cloths treated with maleic acid.

| Sample  | % Add-on <sup>(a)</sup> | Cure Temperature <sup>(b)</sup> | Breaking Strength <sup>(c)</sup><br>(lb.) | DWR <sup>(d)</sup><br>(W+F) |
|---------|-------------------------|---------------------------------|-------------------------------------------|-----------------------------|
| Control | —                       | —                               | 53                                        | 166                         |
| Group A |                         |                                 |                                           |                             |
| 53      | 5.4                     | 160                             | 30                                        | 190                         |
| 55      | 4.3                     | 160                             | 23                                        | 200                         |
| 56      | 6.0                     | 160                             | 27                                        | 200                         |
| 57      | 4.3                     | 160                             | 25                                        | 210                         |
| 59      | 7.7                     | 160                             | 44                                        | 190                         |
| 76      | 4.6                     | 140                             | 38                                        | 158                         |
| 85      | 6.2                     | 140                             | 43                                        | 142                         |
| 86      | 6.6                     | 140                             | 56                                        | 86                          |
| Group B |                         |                                 |                                           |                             |
| 61      | 9.3                     | 160                             | 31                                        | 182                         |
| 72      | 12.9                    | 160                             | 32                                        | 92                          |
| 79      | 10.6                    | 160                             | 45                                        | 94                          |
| 81      | 12.2                    | 140                             | 68                                        | 96                          |
| 82      | 12.1                    | 140                             | 55                                        | 94                          |
| 83      | 9.3                     | 140                             | 46                                        | 100                         |
| 87      | 8.8                     | 140                             | 59                                        | 100                         |
| Group C |                         |                                 |                                           |                             |
| 69      | 24.3                    | 160                             | 47                                        | 56                          |
| 78      | 15.2                    | 140                             | 51                                        | 100                         |

<sup>(a)</sup> Percent add-on represents the total weight gain due to the polyoxymethylene and the crosslinking agent after curing.

<sup>(b)</sup> All samples cured at the given temperature for 15 minutes in a forced-draft oven.

<sup>(c)</sup> ASTM-D1682-64; Average of three runs per sample, warp direction only.

<sup>(d)</sup> ASTM-D1295-60-T; Average of five runs per sample.

TABLE 6

### Some physical properties of polyoxymethylene-coated cotton cloths treated with 1,2,3,4-cyclopentane tetracarboxylic acid<sup>(d)</sup>

| Sample  | % Add-on <sup>(a)</sup> | Breaking Strength <sup>(b)</sup><br>(lb.) | % Elonga-<br>tion <sup>(b)</sup> | DWR <sup>(c)</sup><br>(W+F) |
|---------|-------------------------|-------------------------------------------|----------------------------------|-----------------------------|
| Control | —                       | 53                                        | 5.8                              | 175                         |
| Group A |                         |                                           |                                  |                             |
| 140     | 8.9                     | 35                                        | 5.0                              | —                           |
| 141     | 9.3                     | —                                         | —                                | 185                         |
| 143     | 9.6                     | 29                                        | 5.4                              | —                           |
| 110     | 7.5                     | —                                         | —                                | 199                         |
| 115     | 7.2                     | 43                                        | 6.0                              | —                           |
| 120     | 7.2                     | 42                                        | 5.4                              | —                           |
| 122     | 6.8                     | —                                         | —                                | 188                         |
| Group B |                         |                                           |                                  |                             |
| 111     | 5.5                     | 36                                        | 5.4                              | —                           |
| 112     | 5.5                     | —                                         | —                                | 217                         |
| 113     | 5.6                     | 35                                        | 5.5                              | —                           |
| 114     | 7.5                     | —                                         | —                                | 196                         |
| 116     | 4.8                     | 32                                        | 5.8                              | —                           |
| 119     | 6.2                     | 43                                        | 6.0                              | —                           |
| 121     | 4.3                     | —                                         | —                                | 212                         |

|    |         |     |     |    |     |     |
|----|---------|-----|-----|----|-----|-----|
| 5  | Group C | 118 | 3.3 | 39 | 5.6 | —   |
|    |         | 126 | 3.1 | 32 | 5.1 | —   |
|    |         | 127 | 2.4 | 36 | 5.7 | —   |
|    |         | 128 | 2.6 | 32 | 5.8 | —   |
|    |         | 129 | 3.6 | —  | —   | 230 |
|    |         | 133 | 1.9 | —  | —   | 229 |
| 10 |         | 145 | 2.9 | 39 | 5.5 | —   |
|    |         | 146 | 2.5 | —  | —   | 221 |
|    |         | 147 | 3.2 | 30 | 5.8 | —   |
|    |         | 148 | 2.8 | 36 | 5.9 | —   |

<sup>(a)</sup> Percent add-on represents the total weight gain due to the polyoxymethylene and the crosslinking agent after curing.

<sup>(b)</sup> ASTM-D1682-64; Average of three runs per sample, warp direction only.

<sup>(c)</sup> ASTM-D1295-60-T; Average of five runs per sample.

<sup>(d)</sup> All samples dipped in 2% acid bath for 10 minutes, dried at 80° C., then cured for 20 minutes at 150° C.

TABLE 7.—Some physical properties of polyoxymethylene-coated cotton cloths treated with epichlorohydrin.<sup>1</sup>

| Sample  | Percent add-on <sup>a</sup> | Breaking strength (lbs.) <sup>b</sup> | Percent elongation <sup>b</sup> | DWR <sup>c</sup> (W+F) <sup>c</sup> | WWR <sup>d</sup> (W+F) <sup>d</sup> | Elmendorf tear (Gms.) <sup>e</sup> |
|---------|-----------------------------|---------------------------------------|---------------------------------|-------------------------------------|-------------------------------------|------------------------------------|
| Control | —                           | 53                                    | 5.8                             | 166                                 | 150                                 | 470                                |
| 130     | 1.7                         | —                                     | —                               | 214                                 | 210                                 | 459                                |
| 131     | 1.8                         | —                                     | —                               | —                                   | —                                   | —                                  |
| 132     | 2.6                         | 43.3                                  | 9.3                             | —                                   | —                                   | —                                  |
| 134     | 2.4                         | —                                     | —                               | —                                   | —                                   | 491                                |
| 117     | 1.2                         | 35.9                                  | 7.8                             | —                                   | —                                   | —                                  |
| 155     | .26                         | —                                     | —                               | 172                                 | 208                                 | —                                  |
| 156     | 3.4                         | 43.6                                  | 8.8                             | —                                   | —                                   | 517                                |
| 157     | .50                         | —                                     | —                               | —                                   | —                                   | —                                  |
| 158     | .90                         | —                                     | —                               | 190                                 | 200                                 | —                                  |
| 159     | .80                         | 44.3                                  | 8.5                             | —                                   | —                                   | —                                  |
| 164     | 1.8                         | —                                     | —                               | —                                   | —                                   | 517                                |
| 165     | .33                         | —                                     | —                               | 182                                 | 170                                 | —                                  |
| 166     | .30                         | 37.3                                  | 8.4                             | —                                   | —                                   | —                                  |
| 167     | .12                         | —                                     | —                               | —                                   | —                                   | 512                                |
| 168     | .29                         | —                                     | —                               | 178                                 | 174                                 | —                                  |
| 169     | .60                         | 41.6                                  | 8.4                             | —                                   | —                                   | —                                  |
| 170     | 1.8                         | 41.3                                  | 9.1                             | —                                   | —                                   | —                                  |
| 171     | .98                         | —                                     | —                               | —                                   | —                                   | 501                                |
| 172     | .60                         | —                                     | —                               | 202                                 | 218                                 | —                                  |
| 173     | 2.0                         | 41.8                                  | 8.8                             | —                                   | —                                   | —                                  |
| 174     | 1.5                         | —                                     | —                               | —                                   | —                                   | 560                                |
| 175     | 2.0                         | —                                     | —                               | 192                                 | 212                                 | —                                  |
| 176     | 1.0                         | 45.8                                  | 9.7                             | —                                   | —                                   | —                                  |
| 177     | 1.8                         | —                                     | —                               | —                                   | —                                   | 533                                |
| 178     | 1.7                         | —                                     | —                               | 166                                 | 156                                 | —                                  |
| 179     | 1.2                         | 42.8                                  | 8.8                             | —                                   | —                                   | —                                  |
| 180     | .87                         | 42.0                                  | 8.7                             | —                                   | —                                   | —                                  |
| 181     | .35                         | —                                     | —                               | —                                   | —                                   | 512                                |
| 183     | .85                         | —                                     | —                               | 212                                 | 184                                 | —                                  |
| 184     | 1.0                         | 40.9                                  | 8.0                             | —                                   | —                                   | —                                  |
| 185     | 2.5                         | —                                     | —                               | —                                   | —                                   | 491                                |
| 186     | 2.0                         | —                                     | —                               | 192                                 | 194                                 | —                                  |
| 187     | 3.1                         | 40.8                                  | 8.4                             | —                                   | —                                   | —                                  |
| 188     | 2.3                         | —                                     | —                               | —                                   | —                                   | 528                                |
| 189     | 1.9                         | —                                     | —                               | 192                                 | 198                                 | —                                  |

<sup>a</sup> Percent add-on represents the final weight gain resulting after curing.

<sup>b</sup> ASTM-D1682-64; average of 4 runs per sample, warp direction only.

<sup>c</sup> ASTM-D1295-60-T; average of 5 runs per sample.

<sup>d</sup> ASTM-D1295-60-T; average of 5 runs per sample; samples conditioned for five minutes in 0.1% Triton X-100 solution.

<sup>e</sup> ASTM-1424-63; average of 3 runs per sample, warp direction only.

<sup>f</sup> All samples dipped in 5% NaOH, then 20% epichlorohydrin (both in absolute ethanol), then cured for 10 minutes at 100° C. in a forced-draft oven.

I claim:

1. A process for imparting superior physical properties to a cellulosic textile fabric, comprising:
  - wetting the surface of the cellulosic textile fabric with an alkaline catalyst solution at ambient temperature;
  - applying highly purified anhydrous formaldehyde vapor to the surface of the catalyst-impregnated fabric to produce a fabric with a weight add-on of about 2 to 50 percent of a uniform and essentially continuous oxymethylene polymer surface deposition; and
  - reacting the residual hydroxyl end groups of the oxymethylene polymer of the said surface deposition with a compound selected from the group consisting of acid an-

hydrides, epoxides, chloroalkylethers, and isocyanates, to retard high temperature depolymerization of said continuous oxymethylene polymer.

2. A process for producing a crosslinked cellulosic textile fabric having superior physical properties, comprising:

- a. wetting the surface of the cellulosic textile fabric with an alkaline catalyst solution at ambient temperature;
- b. applying highly purified anhydrous formaldehyde vapor to the surface of the catalyst-impregnated fabric to produce a fabric with a weight add-on of about from 2 to 10 50 percent of a uniform and essentially continuous oxymethylene polymer surface deposition;
- c. reacting the residual hydroxyl end groups of the oxymethylene polymer of the said surface deposition with a compound selected from the group consisting of acid anhydrides, epoxides, chloroalkylethers, and isocyanates to

5

10

15

20

25

30

35

40

45

50

55

60

65

70

75

retard high temperature depolymerization of said continuous oxymethylene polymer;

- d. reacting the oxymethylene polymer-coated fabric of step (c) with a suitably catalyzed solution containing a cross-linking agent selected from the group consisting of methylol derivatives of cyclic ureas, methylol derivatives of melamine, methylol derivatives of urea, and methylol carbamates; and
- e. then washing and drying the resulting oxymethylene polymer-coated and crosslinked fabric to obtain shape-holding properties in the finished fabric.

3. The cellulosic textile product produced by the process of claim 1.

4. The cellulosic textile product produced by the process of claim 2.

\* \* \* \* \*